

June 12, 1923.

A. BONIFACE

1,458,681

SLIP PROOF STAIR UNIT

Filed March 10, 1919



INVENTOR  
*Arthur Boniface*  
BY  
*Clayton L. Jenkins*  
ATTORNEY

## UNITED STATES PATENT OFFICE.

ARTHUR BONIFACE, OF NEW YORK, N. Y., ASSIGNOR TO NORTON COMPANY, OF WORCESTER, MASSACHUSETTS, A CORPORATION OF MASSACHUSETTS.

## SLIPPROOF STAIR UNIT.

Application filed March 10, 1919. Serial No. 281,770.

To all whom it may concern:

Be it known that I, ARTHUR BONIFACE, a citizen of the United States of America, residing at New York, in the county of New York and State of New York, have invented certain new and useful Improvements in Slipproof Stair Units, of which the following is a full, clear, and exact specification.

My invention relates to concrete articles of manufacture and more particularly to the construction of slip-proof stair treads. An efficient and satisfactory stair tread has been found in embedding a tile of ceramic bonded crystalline alumina in the nose of a concrete stair. Considerable difficulty has been experienced in substituting this form of stair tread for the unsafe stairs used, for example, in the approaches to elevated railway structures, since it is not feasible to build a concrete stairway from the plastic material where it is necessary for pedestrians to pass over this surface at frequent intervals.

It is accordingly an object of my invention to overcome such difficulties and to provide as a new article of manufacture a concrete slab having an anti-slipping nose which is adapted to be quickly laid in place on a suitable stair foundation without seriously impeding pedestrian traffic thereover.

Referring to the drawings, I have there illustrated one embodiment of my invention in which:

Fig. 1 is a plan view; and

Fig. 2 is a perspective view of a section of a slab adapted for a stair tread.

My slip-proof stair slab comprises essentially a concrete or cement body having anti-slipping tiles embedded in one face to form a plane tread surface and having a bottom adapted to be laid on a foundation and suitably fastened thereto.

This slab is an integral and unitary article of rigid and strong construction which may be made up in various shapes and designs at some convenient manufacturing establishment and then shipped to a desired location where it may be quickly laid in place on a stair foundation without seriously interrupting pedestrian traffic. This slab may be so constructed that it may be supported and fastened to a stair construction in various ways.

One embodiment of my invention may comprise the construction illustrated in the drawings which is adapted to be supported

on a flat iron stairway and bolted thereto. This slab comprises essentially a concrete body 10 having preferably a cement layer 11 thereover, which is adapted to hold the anti-slipping tiles in place and to form a smooth tread portion for the rear of the slab. The slip-proof tiles 12 which I utilize are preferably in the form of flat plates substantially the shape of a parallelepipedon. Having rough porous surfaces, they may be laid in plastic cement and become securely united thereto as the latter hardens. As a further aid to such union and to overcome any tendency to slip forward or move in the cement, the tiles are preferably provided with grooves 13 in their under surfaces.

Since the pedestrian wear on a stairway occurs mainly on its forward edge or adjacent to the nose and not on the rear and end portions thereof, I embed these tiles only in such forward and middle portions, as shown in Fig. 1. The portions in the rear of the tiles and at the ends of the tread are filled with the cement 11 to provide a rear surface 14 and sides 15 plane and continuous with the top of the tiles.

In order to add further strength to the concrete slab I may provide suitable reinforcement means such as a wire mesh 16 which is embedded in the concrete. It is within the scope of my invention to provide various means for fastening this slab to a support. In the embodiment illustrated this may comprise the bolts 17 having their heads 18 embedded in the concrete and preferably above and engaging the wire mesh 16.

As a simplified type of process for making this concrete stair slab, I may place the tiles 12 in a suitable mold with their tread portions facing downwardly and the round noses 19 toward one corner of the mold, these blocks having been previously wetted with water and permitted to drain somewhat. A layer 11 of cement mortar of one part of Portland cement to one part of sand mixed with water to the proper consistency is filled in the space in the rear of, and to a level about  $\frac{1}{4}$ " above the top of, the tiles and is carefully worked into grooves 13, between the tiles and around the sides in order to give thorough and intimate contact. After this plastic mass has been put in position and before it can harden I pour in the layer 10, which may comprise a regular concrete mixture of one part

of Portland cement, two parts of sand and four parts of aggregate of broken rock, gravel and so forth. The reinforcement 16 comprising a wire network is then suitably 5 located in the concrete mass. The iron bolts 17, adapted for fastening the slab to a stair, are so positioned that their heads lie below the wire mesh in the mold and the stems project outside of the slab. After permitting 10 the cement mixtures to set in the mold for a suitable length of time, the slab is removed and is then ready for use.

The anti-slipping tiles, which are made by methods not forming a part of my invention, may comprise wear-resisting crystalline grains of alumina, silicon carbide or other materials having a hardness of 9 or more on Mohs' scale, which are bonded into a unitary mass by a suitable bond capable 15 of holding these crystalline grains in place almost indefinitely and withstanding the shocks and abrasions of pedestrian foot-wear. Such a bond preferably comprises a ceramic material which is made up of 20 suitable clay mixtures such as slip clay mixed with ball clay and feldspar in such proportions that when burned at about 1300° C., they produce a very hard bonded 25 structure. The grain sizes are such as to prevent slipping of footgear but at the same time are small enough so as not to seriously abrade shoe leather. These grains preferably vary in size from a 36 mesh to very fine grains such as will pass a 120 or 180 mesh screen.

Having thus described my invention, what I claim as new and desire to secure by Letters Patent is:—

A unitary, integral stair slab comprising a supporting portion of cement, a row of 40 wear-resisting, anti-slipping tiles of ceramic bonded abrasive grains forming the forward part of the tread surface of the slab, said tiles being rough and porous and having plane upper surfaces, rounded abrasive edges forming the nose of the slab and under surfaces integrally adhering to the cement, a portion comprising cement in the rear of the tiles having a plane tread level and continuous with the surface of the tiles 45 and a securing device embedded in said slab for fastening it to a foundation.

Signed at New York, N. Y., this 6th day of March 1919.

ARTHUR BONIFACE.